

# UNITED STATES PATENT OFFICE.

FOSTER MILLIKEN, OF LAWRENCE, NEW YORK.

## ALLOY.

1,314,417.

Specification of Letters Patent. Patented Aug. 26, 1919.

No Drawing.

Application filed August 29, 1918. Serial No. 251,941.

To all whom it may concern:

Be it known that I, FOSTER MILLIKEN, a citizen of the United States, and a resident of Lawrence, in the county of Nassau and State of New York, have invented a new and Improved Alloy, of which the following is a full, clear, and exact description.

This invention relates to an alloy, the basis of which is made up of copper, nickel, iron and zinc, with which are mixed certain other metals, whereby the alloy is capable of being rolled, forged, drawn or worked in other ways while the metal is hot. Heretofore alloys of this character, as far as I am aware, have had to be worked by the cold process, that is to say, by annealing from time to time and then working while cold. This alloy can also be worked cold.

In addition to this new alloy being adapted for hot working and cold working it has the further advantage of being highly resistant to acid. The alloy comprises—

|                 |                 |
|-----------------|-----------------|
| Copper -----    | 40-48 per cent. |
| Nickel -----    | 8-12 " "        |
| Zinc -----      | 38-48 " "       |
| Iron -----      | 1-6 " "         |
| Manganese ----- | 1-3 " "         |

A test of the new alloy and cold rolled alloys with a 15 per cent. sulfuric acid solution resulted as follows:

30

|                                | Hot rolled.  | Cold rolled. |
|--------------------------------|--------------|--------------|
| Original weight of sample..... | 21.7280 grs. | 11.6360 grs. |
| Weight one week after .....    | 21.7186 "    | 11.6226 "    |
| Loss in seven (7) days.....    | .0094 "      | .0134 "      |
| Surface exposed .....          | 2.25 sq. in. | 3.15 sq. in. |
| Loss per square inch .....     | .00418 grs.  | .00425 grs.  |

35

I claim:

An alloy consisting of the following ingredients in substantially the following proportions, copper 40-48 per cent., nickel 8-12 per cent., zinc 38-48 per cent., iron 1-6 per cent., manganese 1-3 per cent.

FOSTER MILLIKEN.

40